

W. BUEHLER.

## PRESERVING WOOD

APPLICATION FILED JUNE 6, 1908.

899,480.

Patented Sept. 22, 1908.



# UNITED STATES PATENT OFFICE.

WALTER BUEHLER, OF MINNEAPOLIS, MINNESOTA, ASSIGNOR OF ONE-HALF TO GEORGE W. BESTOR, OF MINNEAPOLIS, MINNESOTA.

## PRESERVING WOOD.

No. 898,480.

Specification of Letters Patent. Patented Sept. 22, 1908.

Application filed June 6, 1908. Serial No. 437,145.

*To all whom it may concern:*

Be it known that I, WALTER BUEHLER, a citizen of the United States, and resident of Minneapolis, Minnesota, have invented certain new and useful Improvements in the Art of Preserving Wood, of which the following is a full, clear, and exact description, such as will enable others to practice the same.

My invention relates to improvements in the art of impregnating wood with preservative liquids.

While not limited thereto the invention is chiefly concerned with the impregnation of seasoned wood with bituminous liquids and distillates of bituminous substances, commonly known as oils, which are substantially free from water, such as creosote oil.

It is now generally conceded that, when properly treated with creosote oil, a seasoned stick retains substantially its maximum strength; as the oil, unlike water, does not enter or weaken the wood fiber; also the durability of the wood is greatly enhanced, by reason of the fact that the creosote oil, occupying the cells and pores of the wood, excludes moisture from the wood fiber and retards and practically prevents the decomposition or rotting thereof and also effectually preserves the wood against the attack of either land or marine insects.

The object of my invention is to enable the effectual preservation of wood by impregnation with preservative liquid, preferably creosote, and to accomplish the desired results and effects without detriment to the wood fiber, within a short space of time and at low cost.

My invention comprises a process, or improvement in the art, of preserving seasoned or partially seasoned wood, which consists in first exhausting the gaseous content of the wood, principally air, and thus creating a vacuum in the wood cells and pores, then immersing the wood in preservative liquid, then by pressure upon the liquid driving the requisite quantity thereof into the cells and pores of the wood, then emersing the wood, *i. e.* withdrawing the surplus liquid, then subjecting the partially impregnated wood to the action of compressed gas, preferably air, thereby driving the liquid into the wood, and then relieving the gas pressure.

My invention as above briefly described,

together with certain desirable incidental steps, thereof will be more readily understood by reference to the accompanying drawing, forming a part of this specification and in which I have illustrated the apparatus that I have found to be best adapted to the purposes of the invention.

In these drawings, 2, represents a cylinder or receptacle of the kind usually employed in preserving wood. This cylinder is large enough to contain a car or truck, 3, and its load of wood, 4. A large door or head, 5, tightly closes the end of the cylinder, the packing being such as to permit a high pressure of liquid or of gas to be maintained in the cylinder. The dotted lines, 6, represent a steam coil which may be and is preferably located within the cylinder.

7 represents a liquid reservoir of capacity exceeding that of the cylinder, 2, and provided with an indicator, 8, for determining the quantity of liquid in or that is withdrawn from the reservoir.

The dotted lines, 9, represent a steam coil which may be and preferably is located in the reservoir, 7.

When creosote oil is used it is usually necessary to heat or warm it, in order to keep it in a liquid state, its temperature of liquefaction approximating 150 degrees Fahrenheit. A pipe or main, 10, connects the reservoir with the cylinder, 2, branches, 10' and 10", being preferably employed at the cylinder. A pump, 11, is used for transferring the liquid from one receptacle to the other and is also preferably used in obtaining the necessary liquid pressure within the cylinder. Suitable valves, 12, 13 and 14 are arranged in the connections, 10, 10', 10". A small boiler, 15, supplies the steam required in the coils, 6 and 9 and is connected therewith by pipes containing the valves, 15', 6' and 9'.

16 is the blow-off connection of the cylinder, containing a valve, 16'. A vacuum pump, 17, is connected with the cylinder by a pipe, 17', containing the controlling valve, 17".

18 represents apparatus for compressing and storing air or other gas for use in the cylinder, being connected therewith by pipe, 18', provided with controlling valve, 18".

19 is a vacuum gage, and 20, a pressure gage, both connected with the cylinder.

My novel process is performed or carried out as follows: Upon the arrival of a load of substantially dry or seasoned wood at the cylinder, the door, 5, thereof is swung open, 5 the loaded car is placed in the cylinder and the door is tightly closed. Meantime the valves, 12, 14, 18" and 16' are closed, to completely close or seal the cylinder. At such time the cylinder is free from liquid, the 10 same having been drained therefrom prior to the opening of the cylinder. After the cylinder is closed the vacuum pump, 17, is started and the vacuum valve, 17", opened to establish communication between the pump 15 and the cylinder. The air is thus removed from the cylinder and, slowly from the wood therein, until a considerable vacuum, usually approximating 20 to 26 inches, is established throughout the wood. This state is readily 20 ascertained by closing the valve, 17", when, if the vacuum gage remains substantially stationary, it indicates that a proper rarefaction has been effected. In this manner the 25 wood is deprived of air and vapors and the cells and pores previously emptied of moisture and sap by the seasoning process are prepared to receive the preserving liquid.

The next step of the process consists in filling the cylinder with liquid from the reservoir, 7. In case the preferred preservative, 30 creosote, is used, it is warmed and liquefied before introduction to the cylinder and when found necessary the body of liquid in the cylinder is kept warm by steam in the coil, 35 6, though preferably no attempt is made to raise the temperature of the preserving liquid above that at which it liquefies. The pump, 11, is preferably used in filling the cylinder with liquid and I prefer to continue the 40 vacuum pump in operation until the liquid rises to the top of the cylinder; the vacuum valve, 17", is then closed.

The operation of the vacuum pump during the filling of the tank is not essential to the 45 success of the process, though desirable, as otherwise the slow destruction of the vacuum by the entrance of the liquid results in slight non-uniformity of the liquid charge in the timbers in the upper and lower part of the cylinder. The difference is not important, 50 but as intimated may be avoided by maintaining the vacuum during the filling operation. Or a small quantity of air may be admitted to the cylinder to reduce the vacuum 55 prior to the entrance of the liquid, this last expedient, however, is objectionable as tending to recharge the timber with air.

The pressure pump, 11, is continued in 60 operation after the cylinder has been filled and is kept in motion until the indicator, 8, shows that the requisite quantity of preservative has been forced into the cells and pores of the wood in the cylinder. A reading 65 is taken from the indicator, 8, at the moment that the cylinder is completely filled

and further movement of the indicator therefore shows the quantity of liquid that is placed in the wood. A liquid pressure approximating one hundred to one hundred and fifty pounds is usually sufficient to drive 70 the charge of liquid into the wood. Being unopposed by air, vapors or liquids within the cells of the wood, the preserving liquid very quickly penetrates the outer pores and cells and the time consumed in thus charging the timber is shorter than in other processes. In actual practice of my process, the 75 period of liquid pressure varies from thirty minutes to an hour or more, according to the character and size of the wood under treatment.

When the indicator, 8, shows that the required amount of liquid has been lodged in the wood, the pump is reversed and the surplus liquid is drained from the cylinder, until 80 the wood is completely emersed. If desired, the valve, 12, may be opened at this time and the operation of the pump supplemented by admitting compressed air to the cylinder.

After withdrawing the surplus liquid from the cylinder, I close the valves, 12 and 14 (all other valves are then closed) and admit gas under pressure from the source, 18. The gas employed is preferably air at normal temperature, in other words cool, and I prefer that the pressure of air in the cylinder shall not exceed twenty-five pounds. This pressure may be maintained either continuously or intermittently by manipulation of the 100 valve, 18". The compressed air penetrates the pores and cells of the wood in the cylinder and ultimately forces the charges of liquid therein further into the sticks, thus distributing the liquid uniformly upon the walls of 105 the cells and pores throughout the wood. In this manner a relatively small quantity of preserving liquid is distributed throughout the cellular structure, forming thereon films which effectually exclude moisture 110 from the wood fiber, thus retaining the full strength of the wood. In practice the air pressure is continued until gaseous equilibrium is established in the wood, a fact indicated by the hand of the pressure gage remaining stationary when the compressed air valve, 18", is closed.

In using creosote, I have noted that the temperature of the wood following the charge of warm liquid is sufficient to maintain the creosote in liquid condition in the pores and cells long enough to permit the inward distribution of the liquid by the compressed air, but in extremely cold weather, it is sometimes necessary to slightly warm the 120 cylinder to prevent the premature solidification of the creosote in the outer pores of the wood.

My preference for the low pressure air or gas indicated above is based upon the fact 130

that air or gas at twenty-five pounds pressure will quietly flow from the wood when the latter is removed from the cylinder without expelling the liquid from the cells and pores thereof. Under high pressure the sudden return of the wood to atmospheric pressure is usually followed by the expulsion of considerable quantities of the preservative, and the quantity expelled being difficult to measure, the accuracy of the process is lost, it being then quite impossible to determine the quantity of liquid remaining in the wood. Low pressure gas or air is quite as effectual as the higher pressures in disseminating the liquid in the wood and when relieved escapes at such low velocity that its force is less than the adhesion between the films of liquid and the cell walls, therefore, no loss or disturbance of the liquid films follows the removal of the wood from the cylinder.

After treatment with the compressed air, as above described, the wood is ready for use and the door of the cylinder being opened, the car is removed therefrom, marking the end of the process.

Having thus described my invention, I claim as new and desire to secure by Letters Patent:

1. The herein described improvement in the art of preserving wood that consists in first exhausting the gaseous content of the wood, then immersing the wood in preservative liquid, then by pressure upon the liquid driving the requisite quantity thereof into the cells and pores of the wood, then removing the surplus liquid from the wood, then subjecting the partially impregnated wood to the action of compressed gas, thereby driving the charge of liquid further into the wood, and then removing the gas pressure, substantially as described.

2. The herein described improvement in the art of preserving wood, that consists in causing a vacuum in the load by exhausting the gaseous content thereof, then immersing the wood in non-aqueous preservative liquid, and by pressure thereon driving the same into the outer pores and cells of the wood until the requisite quantity of liquid is lodged therein; then withdrawing the surplus liquid from the wood; then subjecting the wood to the action of low temperature gas at relatively low pressure, until substantially gaseous equilibrium is established in the wood and then restoring the wood to atmospheric pressure, substantially as described.

3. The herein described improvement in the art of preserving wood that consists in placing the wood in a closed vessel; then exhausting the gaseous content of the vessel and of the wood until gaseous equilibrium at less than atmospheric pressure is established within the pores and cells of the wood; then subjecting the wood to pressure of preservative liquid at approximately atmospheric

temperature, thereby lodging a quantity of the liquid in the outer pores and cells of the wood without materially heating the wood; then drawing off the surplus liquid; then subjecting the wood, still within the vessel, to the action of gaseous pressure until gaseous equilibrium at substantially such pressure is established throughout the wood; thereby disseminating the liquid in the cells and pores of the wood and then relieving the pressure of gas and removing the wood from the vessel, substantially as described.

4. The herein described improvement in the art of preserving seasoned wood that consists in creating a vacuum in and throughout the cells and pores of the wood, then immersing the wood in preservative liquid and by pressure upon the liquid driving the requisite quantity thereof into the outer cells and pores of the wood, then removing the surplus liquid, then subjecting the wood to the action of compressed gas, thereby disseminating the liquid throughout said cells and pores and then permitting the quiet restoration of atmospheric pressure within the wood, substantially as described.

5. The herein described improvement in the art of preserving wood that consists in placing the wood to be treated in a closed vessel, then exhausting the air from said vessel and from the wood therein until a substantial vacuum is obtained throughout the cells and pores of the wood; then filling the vessel with warm, non-aqueous preservative liquid, then exerting pressure upon the liquid until the requisite quantity thereof is lodged in the wood; then drawing off the surplus liquid; then filling the vessel with air under given pressure and maintaining said pressure until equilibrium is established throughout the wood, thereby disseminating said quantity of liquid in the pores and cells of the wood, then relieving the air pressure and finally removing the wood from the vessel, substantially as described.

6. The herein described improvement in the art of preserving seasoned wood that consists in exhausting the air from the wood, thus creating a vacuum in the cells and pores thereof, then injecting a quantity of non-aqueous preservative liquid, then draining off the surplus liquid, then injecting compressed air into the wood until the vacuum therein is destroyed and finally restoring the wood to atmospheric air pressure, substantially as and for the purpose specified.

7. The herein described improvement in the art of preserving wood that consists in first creating a vacuum within the cells and pores of the wood, then, without materially reducing the said vacuum, injecting into the outer cells and pores of the wood a quantity of non-aqueous preservative liquid, then draining the surplus liquid from the wood, then distributing the remaining liquid through-

out the cellular structure by external air pressure assisted by the vacuum within the wood, mean time keeping the preservative in a liquid state by maintaining the temperature thereof, and then reducing, to normal, both the temperature of the wood and the pressure therein, substantially as described.

In testimony whereof, I have hereunto set my hand, this 11th day of May, 1908, in the presence of two subscribing witnesses.

WALTER BUEHLER.

Witnesses:

CHARLES GILBERT HAWLEY,  
JOHN R. LEFEVRE.